

L. ST. D. ROYLANCE.

## ORE REDUCING PROCESS.

APPLICATION FILED JAN. 26, 1915.

1,168,678.

Patented Jan. 18, 1916.

2 SHEETS—SHEET 1.



FIG. 1.



FIG. 2.

Inventor  
Leon St.D. Roylance

Witnesses

M. H. Roach  
Chas. E. Roach

By W. N. Roach, Jr.  
Attorney

L. ST. D. ROYLANCE,  
ORE REDUCING PROCESS,  
APPLICATION FILED JAN. 26, 1915.

1,168,678.

Patented Jan. 18, 1916.

2 SHEETS—SHEET 2.



FIG. 4.



FIG. 3.

Inventor  
Leon St. D. Roylance

Witnesses

M. H. Roach  
Chas. E. Roach

By W. N. Roach, Jr.  
Attorney

# UNITED STATES PATENT OFFICE.

LEON ST. D. ROYLANCE, OF SAN FRANCISCO, CALIFORNIA.

## ORE-REDUCING PROCESS.

1,168,678.

Specification of Letters Patent. Patented Jan. 18, 1916.

Application filed January 26, 1915. Serial No. 4,474.

To all whom it may concern:

Be it known that I, LEON ST. D. ROYLANCE, a citizen of the United States of America, residing at San Francisco, in the county of San Francisco and State of California, have invented certain new and useful Improvements in Ore-Reducing Processes, of which the following is a specification.

10 This invention relates to a method or process of separating and recovering precious metals from their ores.

The objects of the invention are to provide a process which will recover a large percentage of the precious metal from its ore; which will recover the gold from its ore under varying conditions without resorting to the old and well-known methods, such as leaching, roasting, and the like; 20 which will be simple and cheap in its operation; and which will be positive and uniform in its action.

I will now proceed to outline my improved method of extracting such metals, first giving a brief description of the apparatus used which is shown in the accompanying drawings, wherein:

Figure 1 is a plan view of the disintegrator, the top being partly broken away. 25 Fig. 2 is a vertical, longitudinal section of the same. Fig. 3 is a vertical sectional view of the agitator and amalgamator. Fig. 4 is a plan view of the same.

Referring to said drawings by numerals, 30 and first to the disintegrator: A tank 1, of any suitable form and material, is provided with an inner curved wall 2 extending from the top of one end of the tank to a position near the center of the bottom. Said wall 2 is provided with a scouring surface 3 formed of any suitable material, but preferably of concrete or unglazed tile. At the end of said tank opposite that at which wall 2 is placed, is an inwardly projecting wall or 35 partition 4 forming within said tank the compartment 5, said wall 4 terminating near the bottom of said tank to form the slot 6 for a purpose hereinafter explained and described. At a convenient point near the top 40 of said tank is placed a suitable charging port 7 and, near the bottom, a discharge port 8. A man hole 9 of any suitable form is provided in the top of said tank, said man hole being closed with a cover 9<sup>a</sup> and said tank is further provided, at convenient 45 points, with a safety, or escape valve 10, a

pressure gage 11, thermometer 12 and a water or electrolyte gage 13. For the purpose of maintaining a suitable heat steam coil 14, connected to a suitable exterior 50 source of heat supply, is provided at any convenient point within said tank. In one end of said tank, and toward the top thereof, is provided an opening to permit the intake of a pump 15 to communicate with the interior of said tank. Said pump may be of any suitable design but preferably a power driven centrifugal pump is used. The exhaust of said pump 15 communicates through a suitable opening in the end of 55 said tank with the aforementioned compartment 5, formed between the end and bottom of said tank and the afore-mentioned wall or partition 4. Within said tank and arranged in suitably spaced relation are the plates 16, said plates being held in position by the properly insulated rods 17 adapted to engage the openings 18 formed in said plates. The said plates 16 are in communication with a suitable source of electric current supply 19 through the circuit 20 which has interposed therein an automatic quick break pole changing switch 21.

It is of course understood that the plates 60 16 may be put in electrical contact in any manner desired but, by preference, the outer or end plates are connected directly to the circuit 20 thereby forming main electrodes. The plates interposed between these end or outer plates have no metallic connection 65 therewith or with each other the only connecting medium between them being the electrolyte in which they are immersed. These interposed plates will be found when the current is on, to be electrically active the faces thereof becoming anode and cathode to 70 correspond with the cathode and anode face respectively of the plates next in order to them.

The tank so far described is of the closed variety intended more especially for use in those cases where a high degree of heat and a consequent pressure is desirable. For the treatment of substances requiring the ordinary lower temperatures the open form of 75 tank is more convenient. Such tank is, in the main, similar to that described except that the top with its man-hole and other fittings is discarded, as is also the charging 80 port 7. In place of the top 9, the tank is provided with a removable funnel shaped hood 22, shown most clearly in Fig. 2, pro-

vided with the vent or exhaust pipe 23 adapted to carry off the gases arising from the tank. The exhaust pipe 23 is provided with a damper or check valve 24 to control 5 the escape of said gases.

Referring now to the combined agitator and amalgamator, shown most clearly in Figs. 3 and 4:—A suitable tank 25, is provided with a ball bearing gland 26, which 10 supports in any suitable manner, the radially extending arms 27. Arms 27 are provided with suitably spaced discharge nozzles 28 which are inclined toward the bottom of the tank. Tank 25 is further provided in the 15 side wall thereof with an outlet port through which the interior of said tank is placed in communication with the intake of a suitable centrifugal pump 29, by means of pipe 30. The discharge pipe 31, communicates with 20 the ball bearing gland 26. Gate valves 32 and 33 are provided in pipes 30 and 31 respectively, for the purpose of regulating the flow to and from said pump. Suitably spaced metallic plates 34, are placed around 25 said tank near the top thereof said plates being put in contact in any suitable manner and being connected to a suitable source of electrical supply 35, so as to form of said plates anodes. In the bottom of said tank is 30 the amalgamating plate 36 connected, in any suitable manner, to the other side of said source of electrical supply. The ball bearing gland 26, arms 27 and nozzles 28 are also connected to said opposite side of the electrical source, to prevent electrical disintegration of said parts. Before the ore is 35 subjected to my process it goes through the usual preliminary preparation, that is; the gold bearing ore is first crushed through 40 rock breakers and fed to stamp mills or crushers and crushed to about twenty mesh. This crushed ore is then run through ball or tube mills and pulverized to a fineness of about one hundred and 45 fifty mesh. The ore after being so pulverized, is charged into the electro-chemical decomposing tanks, the solution containing the necessary chemicals for producing the 50 chemical reactions by the aid of the electric current is also charged into the tank, the circulation mechanism is set in motion, the electric current applied and the ore is treated electro-chemically for a period of time necessary for the decomposition or oxidization 55 of the pulp; the time being from one to four hours.

To more fully understand the action of the disintegrator, let us take a simple electrolyte, such as water, with enough rock-salt (NaCl) 60 added thereto to sufficiently reduce the resistance to suit the electric current conditions. In the solution, or electrolyte, let us place a pulverized rebellious ore containing gold, silver, arsenic, antimony, zinc, sulfur and iron. The action is as follows: The

water is decomposed, hydrogen (H) being liberated at the negative side of the plates or electrodes and oxygen (O) at the positive. The next reaction is that of the sodium chlorid (NaCl), chlorin is liberated at the 70 anode and hydrogen and sodium hydrate are formed at the cathode. The chlorin is a direct product of electrolysis but not so the hydrogen and sodium hydrate. Metallic sodium is first deposited, and this then reacts on the water of the electrolyte, forming sodium hydrate and liberating hydrogen. 75

It will be noted, from the above, that we have three very active elements; namely hydrogen, oxygen and chlorin, liberated at the 80 faces of the plates and moreover we have them in their nascent and consequently most active state. By the action of the pump we have the various substances contained in the ore swept through the narrow spaces between the electrodes, which spaces contain the nascent and extremely active elements above noted, whose tendency is to unite with the various metals and compounds, to form new compounds, some of which pass off 85 in the form of a gas, while others form compounds or are oxidized into a state capable of being broken up by the scrubbing and scouring action due to the particles impinging upon the abrading surface 90 of the curved wall of the tank. The gold is not deleteriously acted upon by any of the elements or compounds formed within the electrolyte. The silver is but slightly affected by the chlorin as the process of 100 treatment does not exceed four hours.

The antimony combines with hydrogen forming stibin ( $SbH_3$ ), also with chlorin forming antimony trichlorid ( $SbCl_3$ ). The arsenic combines with hydrogen forming 105 arsin ( $AsH_3$ ). The zinc combines with chlorin forming chlorid of zinc ( $ZnCl_2$ ). The sulfur combines with hydrogen forming sulfureted hydrogen ( $H_2S$ ). The iron combines with oxygen to form ferrous oxid 110 ( $FeC$ ) and also with chlorin to form ferrous chlorid ( $FeCl_2$ ).

In addition to the above we have the possibility of forming such compounds as sulfuric acid ( $H_2SO_4$ ) and hydrochloric acid 115 ( $HCl$ ) which are excellent oxidizing agents and are made possible by the circulating action of the agitating pump. After the pulp has undergone this decomposition, or oxidization, the electric current is switched off 120 and the circulating mechanism stopped. The solution is allowed to stand long enough to allow the pulp to settle to the bottom of the tank. The electrolyte is then siphoned 125 off and stored for further use. The pulp being now in a free milling state, is ready for amalgamation except that it shows an acid reaction and, for reasons heretofore set forth, must be neutralized before amalgamation can be attempted. 130

Neutralization may be effected with any suitable alkali; I prefer however to use calcium oxid, commonly known as slaked lime. This not only gives the desired result, but appears to liven the mercury and aid it in its amalgamating action. After neutralizing the pulp it is transferred to the amalgamating agitator, heretofore described to undergo amalgamation. The amalgamating solution is then added to the tank to a point well above the anodes 34. An electric current of sufficient density is applied from a suitable source 35, the positive pole thereof being connected to the anodes 34 and the negative pole to the amalgamating plate 36. The circulating pump is then started, the radial arms 27 are caused to revolve by the discharge from the nozzles 28, the material so discharged impinging upon the amalgamating plate 36. The gold in metallic form will be precipitated upon the amalgamating plate and forced into the film of mercury coating the plate.

It will, of course, be understood that the amalgamating solutions used are selected to suit the chemical conditions of the ore pulp, and the chemicals therein are of such a nature that, when the solution is subjected to the action of an electric current, the chemical reactions are such that the elements that are liberated at the negative pole, or amalgamating plate, are in a nascent state and have great affinity for oxygen,

and combine with the oxygen of the oxidized mercury, forming soluble compounds 35 and tending to keep the mercury free from oxygen, thereby maintaining it in a clean, live and amalgamable state.

It will be seen, from the foregoing, that my process contemplates disintegrating the ore before amalgamation instead of at the time of amalgamation, thereby avoiding the wastes necessary where amalgamation and disintegration take place together, as heretofore, set forth. 45

Having described my invention, what I claim as new and desire to secure by Letters Patent, is:—

1. In an ore reducing process, disintegrating said ore by subjecting the same to 50 electro-chemical action and at the same time scouring said ore, neutralizing the pulp so obtained, and then subjecting said pulp to amalgamation.

2. In an ore reducing process, disintegrating said ore by subjecting the same to electro-chemical action and at the same time scouring said ore, and then subjecting said pulp to amalgamation. 55

In testimony whereof I hereunto affix my 60 signature in presence of two witnesses.

LEON ST. D. ROYLANCE.

Witnesses:

A. J. HENRY,  
F. H. SEARLS.